

Sept. 26, 1961

K. A. METCALFE ET AL

3,001,888

METHOD OF DEVELOPING AN ELECTROSTATIC IMAGE

Filed Sept. 24, 1958



1

3,001,888

## METHOD OF DEVELOPING AN ELECTROSTATIC IMAGE

**Kenneth Archibald Metcalfe, Graymore, South Australia, and Robert John Wright, Hectorville, South Australia, Australia, assignors to The Commonwealth of Australia, care of the Secretary of the Department of Supply, Melbourne, Victoria, Australia**

Filed Sept. 24, 1958, Ser. No. 763,016

Claims priority, application Australia Sept. 25, 1957

5 Claims. (Cl. 117—37)

This invention relates to emulsion developers for electrostatic images.

Development of electrostatic images is at the present time effected principally by three methods, the first of these consisting of the use of dry powders which are dusted onto the image and are subsequently fixed by heating or the like, the second method consisting of the use of a cloud of developer, the third method consisting of the use of liquids which carry the developer material.

It has been shown that there are substantial advantages in using a liquid, as then the pigments or other developer materials are free to move in liquids of selected characteristic and also fixing of the image can take place without added steps such as the heating which was necessary heretofore.

A liquid developer should preferably be of such a nature that, while it allows free movement of the developer materials to the site where they are to be deposited, it should not be dangerous from the viewpoint of fire or explosion. Most of the liquid developers, however, have characteristics such that under suitable conditions they might be inflammable.

The object of the present invention is to improve developers so that this risk can be controlled or entirely removed, a further object being to provide certain improvements to known processes of liquid development such as more rapid development and better means of controlling the density or tone.

In the dry powder development method already known, a cascade principle has been used according to which mechanical objects such as beads are coated with the developer powder and these then apply the powder to the image as they roll over it, such a method having been found very advantageous in methods of dry powder development as the developer is mechanically brought into intimate contact with the image irrespective of some irregularities in the surface.

The present invention also envisages the use of a carrier phase for the developer, but instead of using a solid medium, the carrier is according to our invention a liquid or a gas of such surface tension that the developer can be carried on the surface of its globules and can thereby be deposited onto an electrostatic image as the carrier moves the developer in contact with it.

An emulsion developer for electrostatic images according to our invention can therefore comprise a liquid carrier phase and a liquid developer phase, the liquid carrier phase being immiscible with the liquid developer phase, the liquid carrier phase having a surface tension such that the liquid developer phase is carried on the surface of globules of the said liquid carrier phase when shaken up to produce an emulsion.

According to a more specific form of the invention an emulsion developer for electrostatic images comprises a carrier phase and a developer phase, said carrier phase consisting of a non-inflammable liquid such as water, said developer phase comprising a non-polar liquid having a volume resistivity of not less than  $10^{10}$  ohm-centimeter and a dielectric constant of not greater than three and immiscible with the said carrier phase liquid such as cyclohexane or mineral turpentine or kerosene or xylene,

2

said developer substance having a pigment substance such as phthalocyanine blue suspended in it on the particles of which is a coating forming a control and fixing agent such as a resin or an oil which is only sparingly soluble in the developer liquid or remains deposited on the surface of the pigment substance when the carrier liquid is evaporated whereby, when the liquids are shaken up to produce an emulsion, the globules of the said carrier phase liquid have a film of the developer phase held thereto by ionic attraction but removable therefrom by the field of an electrostatic image.

The importance of this will at once be realized when it is appreciated that an aqueous or non-inflammable developer carrier can be used, it being for instance necessary only to combine a developer with water which, when shaken up, will cause the globules of the water to be coated with the developer.

It will be realized that if for instance a substance such as kerosene is mixed with water, a pigment and bonding medium having previously been incorporated in the kerosene according to the method of preparing liquid developer substances, the two phases namely kerosene and water will not be miscible, and the effect will be to have a separation when the two phases are first mixed together, but when the mixture is shaken the water will be broken up into globules which will be isolated by a film of the kerosene base developer, and the size of these globules can then be controlled by the amount of agitation and in part by the relative ratios of the two phases.

To enable the nature of the invention to be fully appreciated, it will now be described with reference to the accompanying drawings in which:

FIG. 1 is a perspective view in central longitudinal section of a developer tray according to one form of the invention, and

FIG. 2 is a sectional view depicting how the liquid developer phase can be carried across the surface by the liquid carrier phase.

The developer tray depicted in FIG. 1 comprises a tray 1 onto which the paper 2 to be developed is placed, the tray 1 being housed in a casing 3 in which the tray 1 is arranged with a slight downward slope to cause the developer to flow across the tray 1 in one direction.

The casing 3 contains a developer tank 4 which carries in it the developer liquid 5 to the level indicated by 6.

To emulsify the two phases of the liquid developer a pump 7 is provided the rotor 8 of which can be driven in any suitable manner, the pump 7 being connected to the developer tank 4 by an intake duct 9 which allows the developer to flow into the pump, the developer being displaced by the pump flowing up the duct 10 to a two-part duct 11—12, the two-part duct being divided by a directing vane 13 which can be placed either into the position shown in FIG. 1 or which can be swung over towards the left.

The part 11 of the two-part duct is disposed to feed liquid developer displaced by the pump 7 back into the developer tank 4 and when the mechanism is set in the manner indicated, operation of the pump 7 will circulate the two phase developer continually through the tank and in this way will cause the necessary emulsifying of the phases.

The part 12 of the two-part duct leads to a nozzle 14 which extends across the higher end of the tray 1 and has a narrow opening 15 directed across the tray so that when the directing vane 13 is displaced to its opposite position, the emulsified liquid will be drawn from the developer tank 4 by the pump 7 and will be pumped along the path of the dotted arrows in the duct 12 into the nozzle 14 and from there will issue across the paper 2 and the tray 1 in the direction of the dotted arrows, the developer

leaving the tray 1 through the gap 16 between its end and the wall of the developer tank 4.

In this way by appropriately positioning the directing vane 13, the developer can be maintained in an emulsified state by circulating the developer through the pump and the developer tank 4 in the direction of the full line arrows shown in the drawings, and at this stage no flow will take place across the tray 1 from the nozzle 14.

A paper to be developed can then be simply placed into position as shown, preferably by engaging its leading edge into a notch 17 of the tray 1 and the directing vane 13 is then simply swung over to the other position and the emulsified developer will be pumped through the nozzle 14, out of the openings 15 to flow rapidly across the surface of the paper being developed and the tray and back into the developer tank 4, the directing vane 13 being simply swung back to its other position immediately development has been completed which it will be found can take place in a matter of a few seconds, the paper being then simply removed and if an appropriate liquid developer has been used it will be found that the image is dry, or practically dry, the liquid developer phase which coats the aqueous carrier phase globules preventing wetting of the image by water.

It will of course be realized that the actual construction of a mechanism for effecting this could be widely varied and in fact it is not necessary to use a mechanism of the type described as the developer could simply be emulsified by shaking it up in a beaker and immediately pouring it over the paper to be developed.

Referring to FIG. 2 the paper is again represented by the numeral 2 but the liquid phase is designated 20 while the developer phase is designated 21, the globules of the liquid 20 moving the developer phase 21 across the surface 2, it being desirable to have an excess of the developer phase present so that as the film which is held to the water globules by the ionic force, which is less than the electrostatic force on the paper, can be replaced on the surface of the globules during development of an image, for it is found that if insufficient developer is present to maintain a coating on the globules 20, that the globules in contacting the electrostatic image on the paper will tend to destroy the image as they are then not separated by the insulated coating of the developer from the non-insulating water carrier.

The proportion of the developer phase to the carrier phase can be tested by checking to insure that during development sufficient globules are not stripped of their developer coating to allow these to combine and form larger globules.

The following is an example of how the invention may be applied.

#### Developer paste

Fifteen grams of a phenol modified penta-erythritol ester of rosin such as that known under the trade name "Pentarol 20" (acid value 7-15, specific gravity at 20° C. 1.09) is digested in twenty-five grams of xylene and when solution is completed fifteen grams of a linseed oil modified alkyd resin of medium length such as that known under the trade name "Rhodene L6/100" (oil length 52%, acid value 6-10, specific gravity at 20° C., 0.955 to 0.965) is added.

One hundred and fifty grams of phthalocyanine blue is then mixed with the above mixture and blended either in a ball mill or triple roll mill until mixing is complete and pigment particle size is reduced to the required fineness, such as 0.5 micron, average. For the most purpose eight hours milling in a ball mill should be sufficient.

After this it will be found that the pigment particles carry a coating, either continuous or discontinuous, of the coating mix, which will influence the surface charge of the particles and form the bonding means after the pigment is applied in a liquid development process.

#### Paste dispersion

The paste so produced is used as the basis for a dispersion in a liquid of high volume resistivity having a zeta potential greater than the ionic potential of the liquid, dispersion being effected by stirring a small portion of the paste into the required liquid, which in this case may be kerosene, and straining to remove portions of paste that have not completely dispersed.

For fine grain developers filtering should be effected before use.

#### Paste concentration

The concentration of the dispersion may be varied at will but a typical concentration of a preferred dispersion is to utilize 0.5 gram of developer paste in 100 mils of liquid.

#### Carrier liquid

A liquid developer produced in this way, in which particles are coated with a charge controlling and fixing agent which is only sparingly soluble in the high resistivity liquid or remains as a coating for the particles when the liquid of the developer phase is evaporated, is then mixed in the proportion of 100 cc. of the liquid developer to 100 cc. of water, it being then found that the kerosene base developer will be immiscible with the water but on agitation the water will be broken up into globules which will be coated with the liquid developer. The developer is then ready for use in the manner described earlier herein.

#### Globule size

As a guide to the size of the globules these can conveniently range from approximately  $\frac{1}{64}$  of an inch in diameter to  $\frac{1}{8}$  of an inch in diameter although these dimensions are not particularly critical, but it is found that as the globules are of smaller size, the total mixture has a lower volume resistivity with quicker destruction of the electrostatic image during development, the particle size thus affording a degree of control of the time of development, that is the time during which development can take place before the electrostatic image is destroyed by the absorption of developer particles and the presence of the electrically conducting water globules.

Soap emulsifiers and similar material may be used to increase the emulsification provided they are non-ionic, or if ionic, are such that they do not reduce the volume resistivity of the mixture below  $10^{10}$  ohm-centimeter or the dielectric constant above three. Examples of these are gum-arabic, selenium derivatives, glycol and permanganate.

It will be realized that with a water emulsion as described, the danger of fire can be materially reduced or completely eliminated because of the addition of the non-inflammable substance to the inflammable substance, and in this way a developer is provided which not only has improved developing properties but also materially reduces any fire hazard which might otherwise be present, although in practice it has been found that fire risk is negligible even with a carrier base of relatively inflammable liquid.

It will be obvious of course that other carriers than water can be used and it is interesting to note that apart from the reduction of fire hazards there is also a substantial reduction of toxicity if the developers should have this characteristic because the total volume of the emulsion developer contains a correspondingly smaller volume of the developer substance.

An effect of these developers is as said, to give good tone control, as the developer phase can have certain electrical characteristics, whereas the carrier phase can have other characteristics, and by varying the characteristics of particularly the carrier phase it is possible to regulate the rate of bleed-off of the image charge for toning purposes. Similarly the thickness of the developer coating on the

carrier globules, and the resistivity of the developer liquid itself will provide further control means.

From the foregoing it will be realized that the present invention resides in the use of a developer which forms the ~~one~~ phase, the other phase being a substance which is not miscible with the developer so that the developer serves to coat globules of the carrier, which, as said, can then act mechanically to convey the developer to the site, while at the same time controlling the rate of bleed-off of the image charge and serving to reduce or counter the inflammability of the usually more volatile liquid which forms the suspending medium for the pigment and the fixing resin or oil or other substance.

The fact that the globules of the carrier phase have deformable walls allows them to accommodate themselves more readily to surface inequalities in the medium being developed and thus greatly improves the process over the dry developer and rigid bead system.

It will be clear that the developer must be prepared to insure that the developer material such as pigment, remains in the outer phase where it will be the contacting medium when the developer is in use, but this can readily be achieved by first suspending the pigment and resin or other bonding agent in a liquid of suitable high electrical resistivity and then adding the liquid or gaseous carrier phase which, on agitation, will form the carrier globules with the developer coating surrounding same.

To develop an electrostatic image according to this process, the emulsion developer so formed is simply contacted with the image, and the coated pigment particles which are free to move in the liquid, deposit on those areas of the image where a suitable potential exists, until the charge of the image has been satisfied by the particles deposited, the particles being held in position by the electrical force until the carrier liquid is evaporated, whereupon the pigment particles are held by direct adhesion of the resin or other bonding substance on the surface of the particles.

In the case of a developer as specifically described herein, the presence of the resin influence the particle charge, and it is found that rapid deposition of the particles is possible when they are so coated.

The coating mix, according to the example is only partly soluble in the carrier liquid, and therefore, while the partly dissolved surface of the coating is in a condition where it will form an effective bonding medium after evaporation of the solvent, it will act as a surface charge modifier during development to control the migration of the particals in an electrical field.

The developer of the example can be modified by re-

placing the "Rhodene L6/100" with an equal percentage of "Pentarol 20," whereupon it will be found that the developer will have good fixing qualities but will not have the same degree of modification of the surface charge of the pigment particles as the "Pentarol 20" is relatively soluble in the carrier liquid and is a tacky substance, so that it tends to leave the pigment particles when in the developer and deposit as a fixing substance.

If sufficient is present on the pigment substances to cause it to remain there during development, the developer can be said to have both a charge modifying agent and a fixing agent.

The developer can also have the "Pentarol 20" replaced by an equal percentage of "Rhodene L6/100" a substance less soluble in the carrier liquid specified and the developer then acts as one with a high degree of control of the surface charge of the pigment particles due to the coating substance remaining on the pigment particles with possibly even so little solubility on the surface that no appreciable binding of the particles will take place after evaporation of the carrier liquid.

What we claim is:

1. A method of developing an electrostatic image which comprises applying to a body having a latent electrostatic image thereon an emulsion formed by: mixing a pigment in a liquid to form a developer and placing the developer in a carrier liquid with which the developer is immiscible to form an emulsion of the developer and carrier liquid in which the developer coats globules of said carrier liquid.

2. A method as defined in claim 1 wherein said carrier liquid is non-inflammable.

3. A method as defined in claim 1 wherein the amount of developer used is controlled in order to control in turn communication between the globules in the emulsion whereby the image is controllably bled off.

4. A method as defined in claim 1 wherein the carrier liquid is water and the liquid of the developer is kerosene.

5. A method as defined in claim 1 further comprising continuously mixing the carrier liquid and developer and applying the resulting emulsion to said body.

#### References Cited in the file of this patent

#### UNITED STATES PATENTS

|           |              |               |
|-----------|--------------|---------------|
| 1,545,870 | Wyllie       | July 14, 1925 |
| 2,171,851 | Kipper       | Sept. 5, 1939 |
| 2,537,055 | Hiron et al. | Jan. 5, 1951  |
| 2,877,133 | Mayer        | Mar. 10, 1959 |